



US005935368A

# United States Patent [19]

Tingley

[11] Patent Number: 5,935,368

[45] Date of Patent: Aug. 10, 1999

[54] **METHOD OF MAKING A WOOD STRUCTURAL MEMBER WITH FINISHED EDGES**

[76] Inventor: **Daniel A. Tingley**, 3310 SW. Willamette Ave., Corvallis, Oreg. 97333

[21] Appl. No.: **09/024,945**

[22] Filed: **Feb. 17, 1998**

## Related U.S. Application Data

[62] Division of application No. 08/647,181, May 9, 1996, Pat. No. 5,747,151.

[51] **Int. Cl.<sup>6</sup>** ..... E04C 3/29; B32B 5/08

[52] **U.S. Cl.** ..... 156/267; 156/154; 156/166

[58] **Field of Search** ..... 156/154, 166, 156/180, 267, 250

## [56] References Cited

### U.S. PATENT DOCUMENTS

5,026,593 6/1991 O'Brien .  
5,362,545 11/1994 Tingley ..... 156/154 X  
5,456,781 10/1995 Tingley .

### FOREIGN PATENT DOCUMENTS

224050 2/1990 New Zealand .

*Primary Examiner*—Jeff H Aftergut  
*Attorney, Agent, or Firm*—Stoel Rives LLP

## [57] ABSTRACT

A method of manufacturing a glue laminated structural wood member for bearing a structural load includes bonding together multiple elongate wood segments and a synthetic fiber reinforcement with their lengths generally aligned with the length of the member. The synthetic fiber reinforcement includes multiple synthetic fiber strands held within a resin matrix and low cost fiber edges.

**13 Claims, 2 Drawing Sheets**







**METHOD OF MAKING A WOOD  
STRUCTURAL MEMBER WITH FINISHED  
EDGES**

This application is a division of U.S. patent application Ser. No. 08/647,181, filed May 9, 1996, now U.S. Pat. No. 5,747,151, which is hereby incorporated by reference.

**FIELD OF THE INVENTION**

The present invention relates to wood structural members and, in particular, to methods of manufacturing glue laminated wood structural members.

**BACKGROUND OF THE INVENTION**

Beams, trusses, joists, and columns are the typical structural members that support the weight or loads of structures, including buildings and bridges. Structural members may be manufactured from a variety of materials, including steel, concrete, and wood, according to the structure design, environment, and cost.

Wood structural members are now typically manufactured from multiple wood segments that are bonded together, such as in glue-laminated members, laminated veneer lumber and I-beams. They can also be manufactured with wood fibers in a polymer matrix such as parallel strand timber or orientated strand board. These manufactured wood structural members have replaced sawn lumber or timbers because the former have higher design limits resulting from better inspection and manufacturing controls. Wood is a desirable material for use in many structural members because of its various characteristics, including strength for a given weight, appearance, cyclic load response, and fire resistance.

In any application, a load subjects a structural member to both compressive and tensile stresses, which correspond to the respective compacting and elongating forces induced by the load on opposite sides of the member. By convention, a neutral plane or axis extends between the portions of the member under compression and tension. The structural member must be capable of bearing the compressive and tensile stresses without excessive strain and particularly without ultimately failing.

Reinforcement of wood structural members in regions subjected to tensile stresses are known. For example, U.S. Pat. No. 5,026,593 of O'Brien describes the use of a thin flat aluminum strip to reinforce a laminated beam. The use of a synthetic tension reinforcement having multiple aramid fiber strands held within a resin matrix adhered to at least one of the wood segments in the tension portion of the structural member is described by the inventor of the present application in "Reinforced Glued-Laminated Wood Beams" presented at the 1988 International Conference on Timber Engineering.

U.S. Pat. Nos. 5,362,545 and 5,456,781 of Tingley describe methods of adhering the reinforcement to wood using conventional non-epoxy adhesives.

Manufacture of the above-mentioned reinforced structural members results in a significant amount of waste of the relatively expensive synthetic reinforcement material. This waste is generally the result of the planing process to produce a finished edge. Additionally, planing the synthetic reinforcement fiber strands causes significant wear on the cutting tools. Therefore, a need exists for a method of producing structural wood members with synthetic reinforcements without significant waste of the synthetic reinforcement material. Furthermore, a need exists for a method

of producing a finished edge on a structural wood member without significant wear of the cutting tools.

**SUMMARY OF THE INVENTION**

An object of the present invention is, therefore, to provide a method of manufacturing reinforced wood structural members with synthetic fiber reinforcement.

Another object of this invention is to provide such a method that allows efficient application of a synthetic reinforcement to wood structural members.

Still another object of this invention is to provide such a method that provides a synthetic reinforcement with low cost fiber edges.

15 A further object of this invention is to provide such a method that prevents waste of high strength synthetic reinforcement.

20 Yet another object of this invention is to provide such a method that reduces wear of the cutting tools.

25 In a preferred embodiment, the present invention includes a method of manufacturing glue laminated wood structural members in which multiple elongate wood segments and at least one synthetic fiber reinforcement are bonded together with their lengths generally aligned. However, the method would apply to all forms of wood and wood composites from solid wood to plywood to parallel strand lumber. The synthetic fiber reinforcement includes multiple synthetic fiber strands having a high modulus of elasticity in tension and/or compression held within a resin matrix. These fiber strands are relatively high in cost. The edges of the reinforcement are formed from low cost fibers made of material such as hemp, cotton or polyester. The assembled wood member has a width formed by the rough edges of the laminae. The synthetic fiber reinforcement is formed with a width that is substantially matched to the rough width of the wood member. The rough edges are then planed to form a finished width. Only the low cost fiber edges of the reinforcement are planed away avoiding waste of the high cost synthetic fiber strands. Additionally, the low cost fiber edges 30 cause less wear on the cutting tools. Therefore, the low cost fiber edges substantially reduce cost, reduce machinery wear, and improve overall manufacturing ease.

35 Additional objects and advantages of this invention will be apparent from the following detailed description of preferred embodiments thereof which proceeds with reference to the accompanying drawings.

**BRIEF DESCRIPTION OF THE DRAWINGS**

40 FIG. 1 is an elevation view of an exemplary glue laminated structural wood member having a synthetic fiber reinforcement according to the present invention.

45 FIG. 2 is a perspective view of a section of synthetic tension reinforcement with portions cut away to show the alignment and orientation of the fibers.

50 FIG. 3 is a perspective view of a section of synthetic compression reinforcement with portions cut away to show the alignment and orientation of the fibers.

55 FIG. 4 is a perspective view of a pultrusion apparatus for producing an elongate synthetic reinforcement of the present invention.

**DETAILED DESCRIPTION OF PREFERRED  
EMBODIMENTS**

60 FIG. 1 shows a glulam wood structural member 10 having multiple wood laminae 12 that are bonded together and are

preferably elongate boards. In this configuration, glue laminated wood member **10** is configured as a glue-laminated timber according to manufacturing standards 117-93 of the American Institute of Timber Construction (AITC) of Englewood, CO.

A typical structural use of glue laminated wood member **10** is to extend as a beam over and bear a load along an otherwise open region. As a simplified, exemplary representation of such use, glue laminated wood member **10** is shown with its ends supported by a pair of blocks **14** and bearing a point load **16** midway between blocks **14**. It will be appreciated, however, that glue laminated wood member **10** of the present invention could also bear loads distributed in other ways (e.g., cantilevered) or be used as a truss, joist, or column.

Under the conditions represented in FIG. 1, a lowermost lamina **20** is subjected to a substantially pure tensile stress, and an uppermost lamina **22** is subjected to a substantially pure compressive stress. To increase the tensile load-bearing capacity of glue laminated wood member **10**, at least one layer of synthetic tension reinforcement **24** is adhered between lowermost lamina **20** and a next adjacent lamina **26** or, alternatively, to only an outer surface **28** of lowermost lamina **20**. To increase the compressive load-bearing capacity of glue laminated wood member **10**, at least one layer of synthetic compression reinforcement **30** is adhered between uppermost lamina **22** and a next adjacent lamina **32** or, alternatively, to only the outer surface **34** of uppermost lamina **22**. Synthetic reinforcements **24** and **30** are described below in greater detail.

Synthetic tension reinforcement **24** and synthetic compression reinforcement **30** are generally centered about load **16** and preferably extend along about two-fifths to three-fifths the length of wood structural member **10**, depending on load **16**. It can also extend the full length of the wood structural member **10**. A pair of wood spacers **35** are positioned at opposite ends of synthetic tension reinforcement **24** between laminae **20** and **26** to maintain a uniform separation therebetween. Similarly, a pair of wood spacers **35** are positioned at opposite ends of synthetic compression reinforcement **30** between laminae **22** and **32** to maintain a uniform separation therebetween.

General aspects of the process for manufacturing of glue laminated structural wood member **10** are the same as the process for manufacturing conventional glue laminated structural wood members. With regard to the manufacture of conventional glue laminated structural wood members, wood laminae are carried by a conveyor through a glue spreader, which applies multiple thin streams of adhesive (e.g., resorcinol) along the length of each wood lamina on one of its major surfaces.

Wood laminae are successively aligned with and set against other wood laminae in a stack that may be oriented horizontally or vertically. The wood laminae are arranged so that the adhesive on the major surface of one wood lamina engages the bare major surface of an adjacent wood lamina. After all the wood laminae are aligned with and set against each other, pressure in the range of about 125-250 psi is applied to the stack and the adhesive allowed to cure. As is known in the art, sufficient pressure is applied to establish consistent gluelines between adjacent wood laminae **12** of no more than 4 mils (0.10 mm) thick. The edges of the adhered stack of wood laminae **12** are then planed to a finished width so that the sides of all wood laminae **12** are exposed to form a conventional glue laminated structural wood member. This function can be performed by sawing as well.

In a first preferred embodiment, synthetic fiber reinforcements **24** and **30** are carried through a conventional glue spreader (not shown), which applies multiple thin streams of adhesive (e.g., resorcinol) along the length of each reinforcement **24** or **30** on one of its major surfaces. Adhesion between wood laminae **12** and reinforcements **24** or **30** can be relatively poor when the adhesive is applied in the conventional manner. Adhesion is improved, however, when the adhesive is spread to generally completely cover the major surfaces of synthetic fiber reinforcements **24** and **30**. Alternate adhesives are also satisfactory, such as, for example, epoxy adhesives.

It will be appreciated that such spreading of the adhesive can be accomplished by spreading the adhesive applied to one of the major surfaces of synthetic fiber reinforcements **24** and **30** or by spreading the adhesive applied to one of the major surfaces of a wood lamina to be applied to one of synthetic fiber reinforcements **24** and **30**. The spreading of adhesive may be accomplished, for example, by manually spreading the adhesive before synthetic fiber reinforcements **24** and **30** and adjacent wood laminae **12** are engaged or by engaging them and sliding them against each other before the adhesive sets.

During manufacture of the wood member **10**, different wood laminae **12** are successively set against each other with synthetic fiber reinforcements **24** and **30** positioned as desired to form a stack. The stack may be oriented horizontally or vertically so that the sides of adjacent wood laminae and synthetic reinforcements are aligned. Since the laminae **12** and the reinforcements **24** and **30** have substantially the same widths it is not necessary to secure reinforcements **24** and **30** to the stack with pin nails or banding as in previous reinforced wood members. Thus, the time and expense of assembling the stack is reduced.

Preferrably, synthetic fiber reinforcements **24** and **30** are manufactured with respective rough widths **42** and **44** (FIGS. 2 and 3) that are substantially matched to the rough width of wood member **10** (extending into the plane of FIG. 1). Thus, the widths **42** and **44** of synthetic fiber reinforcements **24** and **30** have substantially the same original width as the wood laminae **12** used to form wood member **10**. The original widths of wood laminae **12** used to form wood member **10** can vary so long as they are greater than the finished width of wood member **10**. The original reinforcement width can be the average of these rough widths or whatever is suitable for conditions.

FIG. 2 is an enlarged perspective view of a preferred synthetic tension reinforcement **24**. The tension reinforcement **24** has a large number of synthetic fibers **52** that are arranged substantially parallel to one another and parallel to the longitudinal axis of the reinforcement **24**. The fibers **52** have a relatively high moduli of elasticity in tension and may be made of, for example, an aramid or high performance polyethylene or fiberglass, having a modulus of elasticity in tension in a range of about  $10 \times 10^6$  psi (69,000 Mpa) to about  $33 \times 10^6$  psi (230,000 Mpa). These fibers **52** are generally high cost fibers and it is desirable to prevent waste of these fibers during planing of the wood member **10** to form finished edges.

In order to prevent planing away of the high cost fibers **52** the edges **54** of the tension reinforcement **24** are formed from low cost cotton, hemp, and/or polyester fibers **56**. For illustration purposes, the fibers **56** are shown as having a slightly larger diameter than the fibers **52**. However, it is to be understood that the diameters of fibers **56** and **52** may or may not be the same. Only the outer longitudinal edges **54**

are formed of the low cost fibers **56**. These fibers **56** fill out the die or pack out the reinforcement profile during the pultrusion process to maintain packing fiber matrix volume ratios, alignment, and prevention of fiber crossover or roll-over when the reinforcement is produced.

A resin material **58** surrounds and extends into the interstices between the low cost fibers **56** and the high cost fibers **52** to maintain them in their arrangement and alignment. The fiber/resin volume ratio of the reinforcement **24** is within a range of about 60 percent fibers/40 percent resin to about 83 percent fibers/17 to 40 percent resin. The reinforcement **24** has a composite modulus of elasticity in tension in a range of about  $6 \times 10^6$  psi (41,000 Mpa) to about  $20 \times 10^6$  psi (138,000 Mpa). To facilitate adhesion to the wood laminae **12**, the reinforcement **24** is preferably manufactured and treated as described in U.S. Pat. No. 5,362,545 so that material from the fibers closest to a major surface of the reinforcement protrude from the resin. This may be done by abrading the surface with an abrasive in a direction transverse to the longitudinal direction of the reinforcement.

Alternatively, the surface may be subject to a chemical treatment prior to curing the resin causing voids in the surface which remove portions of the resin and exposes the fibers. Other methods of surface treatment may include the use of broken rovings which protrude from the resin after curing or the use of an epoxy-type of adhesive to achieve sufficient bond strength.

The original or rough edges of the wood member **10** are then planed to produce a finished edge using a high speed cutting tool. Prior synthetic reinforcements are generally formed of one or two types of high cost synthetic fibers, such as, for example, fibers **52**. When the reinforcement is planed to form finished edges, the fibers are cut away and wasted. Since these fibers are generally costly, it is desirable to plane away as little of this material as possible. Preferably, none of the high cost fiber material is planed away. Additionally, such fibers cause machinery wear which further increases cost and decreases efficiency.

When the wood structural member **10** is formed the edges are planed to the finished width. The majority of material planed away is from the low cost fiber edges of the reinforcements **24** and **30**. The amount of material removed from each edge of the wood member **10** during planing is generally in the range of about 0.125 inches to about 0.5 inches. Therefore, each edge **54** preferably has a width **60** within this range. As a result, planing away of the high cost synthetic fibers **52** is avoided. Additionally, the modulus of elasticity of the low cost fibers **56** is generally less than 500,000 psi (3450 Mpa). The fibers **56** are readily machinable with conventional cutting tools, such as, for example, high speed steel planer knives. Forming the edges **54** with the low cost fibers **56** helps prevent waste of the high cost fibers **52**, reduces machinery wear, and increases manufacturing effectiveness.

FIG. 3 is an enlarged perspective view of a preferred synthetic compression reinforcement **30**. The compression reinforcement **30** has a large number of synthetic fibers **62** that are arranged substantially parallel to one another and to the longitudinal axis of the reinforcement **30**. These fibers may be commercially available carbon and fiberglass fibers, which have a modulus of elasticity in compression in the range of about  $34 \times 10^6$  to  $36 \times 10^6$  psi (234,000–248,000 Mpa). The reinforcement **30** is manufactured substantially the same as reinforcement **24** but may include a combination of additional fibers **64** of aramid or high performance polyethylene. The fibers **62** and **64** may be layered or

co-mingled. The edges **66** of reinforcement **30** are formed of low cost fibers **67** similar to fibers **56** in reinforcement **24**. Resin **68** extends between the interstices of the fibers **62**, **64** and **67** to maintain alignment of the fibers. The edges **66** have a width **70** in the range of about 0.125 inches to about 0.5 inches. Synthetic compression reinforcement **30** has a fiber/resin volume ratio within a range of about 60 percent fibers/40 percent resin to about 83 percent fibers/17 percent resin. The reinforcement **30** has modulus of elasticity in compression in the range of about  $18 \times 10^6$  to  $19 \times 10^6$  psi (124,000–131,000 Mpa).

The resin material **58** and **68** used in fabrication of both reinforcement **24** and reinforcement **30** is preferably an epoxy resin, but could alternatively be other resins such as polyester, vinyl ester, phenolic resins, polyimides, or polystyrylpyridine (PSP) or thermoplastic resins such as polyethylene terephthalate (PET) and nylon-66.

Synthetic fiber reinforcements **24** and **30** may be fabricated by various methods, such as a sheet forming or pull-forming process which. Preferably, the reinforcements **24** and **30** are fabricated by pultrusion, which is a continuous manufacturing process for producing lengths of fiber reinforced plastic parts. Generally, pultrusion involves pulling flexible reinforcing fibers through a liquid resin bath and then through a heated die where the reinforced plastic is shaped and the resin is cured. Pultruded parts typically have longitudinally aligned fibers for axial strength and obliquely aligned fibers for transverse strength. In accordance with the present invention, however, preferred reinforcements **24** and **30** are manufactured with substantially all respective fibers in a parallel arrangement and longitudinal alignment to provide maximal strength. In some circumstances, such as to enhance shear resistance in reinforcements **24** and **30**, less than substantially all of respective fibers **52** and **62** would be in a parallel arrangement and longitudinal alignment.

FIG. 4 shows a preferred pultrusion apparatus **72** for fabricating synthetic fiber reinforcements **24** and **30**. Multiple bobbins **74** carry synthetic fiber rovings **76**. As is known in the art, filaments are grouped together into strands or fibers, which may be grouped together into twisted strands to form yarn, or untwisted strands to form rovings. Rovings **76** are fed through openings **78** in an alignment card **80** that aligns that rovings **76** and prevents them from entangling. Openings **78** are typically gasketed with a low friction material, such as a ceramic or plastic, to minimize abrasion or resistance to rovings **76**.

In the fabrication of the reinforcements **24** and **30**, it is understood that the bobbins **74** containing different fibers are constructed and arranged so that as the various fibers exit the card **80** they are arranged to form the reinforcement profiles as shown in FIGS. 2 and 3.

Rovings **76** pass from card **80** to a first comb **82** that gathers them and arranges them parallel to one another. Rovings **76** then pass over a tensioning mandrel **84** and under a second alignment comb **86**. They pass through close-fitting eyelets **88** directly into a resin bath **90** where they are thoroughly wetted with resin material. Passing rovings **76** into resin bath **90** through eyelets **88** minimizes the waste of rovings **76** whenever the pultrusion apparatus **72** is stopped. Resin-wetted rovings **76** are gathered by a forming die **92** and passed through a heated die **94** that cures the resin material and shapes the rovings **76** into reinforcements **24** and **30**. Multiple drive rollers **96** pull the reinforcements **24** and **30** and rovings **76** through pultrusion apparatus **72** at a preferred rate of 3–5 feet/minute (0.9–1.5 m/minute).

To minimize waste and simplify handling and use, the reinforcements **24** and **30** are formed so as to be wound onto a reel (not shown) so that arbitrary lengths can be drawn and cut for use. The reinforcements **24** and **30** are formed with relatively small thicknesses of about 0.25 cm to about 6.4 cm (0.010 in.–0.0250 in.) and can be wound onto reels having a diameter in the range of about 99 cm to about 183 cm (39 in.–72 in.).

Pultrusion apparatus **72** is capable of forming synthetic reinforcements **24** and **30** without longitudinal cracks or faults extending through and with cross-sectional void ratios of no more than 5 percent. Cross-sectional void ratios refer to the percentage of a cross-sectional area of synthetic reinforcements **24** and **30** between respective fibers **52** and **62**, typically occupied by resin material, and is measured by scanning electron microscopy. The absence of faults and the low void ratios assure that synthetic reinforcements **24** and **30** are of maximal strength and integrity.

The preferred resin materials, as described above and applied to rovings **76**, have a glass transition temperature within a range of 250–300° F. Glass transition is an indicator of resin flexibility and is characterized as the temperature at which the resin loses its hardness or brittleness, becomes more flexible, and takes on rubbery or leathery properties. A glass transition temperature within the preferred range is desirable because it provides a minimal fire resistance temperature. The preferred cure rate of the resin material, which is the amount of material that cures from a monomer structure to a polymer structure, is 78 to 82 percent. It has been determined that synthetic reinforcements **24** and **30** with cure rates within this range have higher shear stress bearing capabilities at interfaces with both synthetic reinforcements and wood laminae.

Preferably, a fiber tension force in the range of about three to eight pounds is applied to rovings **76** during the resin cure. The fiber tension force may be applied as a back pressure by tensioning mandrel **84** in combination with combs **82** and **86** or by the use of friction bobbins **74**, wherein rotational friction of the bobbins may be adjusted to provide the desired back pressure on rovings **76**. Such tension in the fibers assists in maintaining their parallel arrangement and alignment in reinforcements **24** and **30**. Also, by curing the resin material while the fibers are under tension, reinforcements **24** and **30** have greater rigidity and therefore decrease deflection of wood member **10** upon loading.

It will be obvious to those having skill in the art that many changes may be made to the details of the above-described embodiment of this invention without departing from the underlying principles thereof. The scope of the present invention should be determined, therefore, only by the following claims.

I claim:

1. In a method of manufacturing a wood structural member for bearing a structural load, the wood structural member having a longitudinal axis and a finished width upon completion of manufacture, the improvement comprising: bonding a synthetic reinforcement having plural tension fiber strands held within a resin matrix to the wood structural member, the plural fibers including different types of fibers wherein one type of fibers form outer side edges of the synthetic reinforcement with the other type of fibers forming the remaining portion of the synthetic reinforcement, the synthetic reinforcement having a reinforcement width greater than that of the finished width of the wood structural member; and reducing the wood structural member and the synthetic reinforcement to the finished width.
2. The method of claim 1 in which the wood structural member includes multiple synthetic reinforcements each of which having two major surfaces, the major surfaces of any one of the synthetic reinforcements not contacting a major surface of any other of the synthetic reinforcements.
3. The method of claim 2 in which the synthetic reinforcements have lengths and the wood structural member has a length, the lengths of multiple ones of the synthetic reinforcements being less than the length of the wood structural member.
4. The method of claim 2 in which one of the synthetic reinforcements includes multiple layers of fiber strands held within the resin matrix.
5. The method of claim 2 in which the fiber strands are selected from a group consisting essentially of carbon, aramid, and high modulus polyethylene with low strength, low cost fibers of cotton, hemp, and polyester forming the outside edges of the synthetic reinforcement.
6. The method of claim 2 in which the bonding of a synthetic reinforcement to the wood structural member is accomplished by applying an adhesive.
7. The method of claim 6 in which the adhesive is a nonepoxy.
8. The method of claim 6 in which the adhesive is resorcinol.
9. The method of claim 6 in which the adhesive is epoxy.
10. The method of claim 1 in which the wood structural member is of a structural composite lumber type.
11. The method of claim 10 in which the structural composite lumber members are selected from a group consisting essentially of laminated wood, laminated veneer wood, parallel strand wood, and I-beam.
12. The method of claim 1 in which the resin matrix is a thermoset resin.
13. The method of claim 1 in which the resin matrix is a thermoplastic resin.

\* \* \* \* \*